

# UNITED STATES PATENT OFFICE.

JULIUS A. C. FICHTMUELLER, OF NEW YORK, N. Y., ASSIGNOR TO DIAMOND DECORATIVE LEAF COMPANY, OF STAPLETON, STATEN ISLAND, NEW YORK, A CORPORATION OF NEW YORK.

## DECORATIVE METALLIC LEAF.

1,160,979.

Specification of Letters Patent.

Patented Nov. 16, 1915.

No Drawing.

Application filed October 18, 1913. Serial No. 796,073.

To all whom it may concern:

Be it known that I, JULIUS A. C. FICHTMUELLER, a citizen of the United States, and resident of the borough of Richmond, county of Richmond, city and State of New York, have made a certain new and useful Invention Relating to Decorative Metallic Leaf, of which the following is a specification.

This invention relates to non-oxidizing or non-staining metallic decorative leaf preferably comprising powdered aluminum or other metallic coloring matter of such character as to be permanent against leather compositions or other action to which such artificial gold leaf or the like is subject under conditions of use. Artificial gold leaf may be made in this way by spraying or otherwise applying to a sized backing or other suitable support such as glass, polished metal, etc., in some cases, a layer of binding material comprising besides volatile solvents and dissolved colloidal protective material, suitable yellowish tinting material and incorporated powdered aluminum or other suitable metallic coloring matter, the leaf being preferably allowed to dry slowly enough so as to effect the stratification of the dissolved tinting and protective material adjacent the sized backing so as to form a glazed protective layer acting to tint to the desired gold color the aluminum powder which seems to stratify in the other side of the layer giving the leaf a silvery metallic luster when viewed from that side.

It is desirable to use the yellowish or orange coloring matter for the tinting material employed in making artificial gold leaf of this description and the tinting material should preferably have sufficient permanence to resist the action of light and other influences to which it is naturally exposed. Suitable tinting materials for this purpose are naphthalene yellow, auramin, aurin, alcohol yellow, gum gamboge, dragon's blood or the like, one or more of these tinting materials being employed in such amounts as to give the desired tinge or shade to the metallic luster leaf, more being of course used for deep gold leaf than for the light gold artificial leaf which is also used for decorative purposes. The tinting ma-

terial is dissolved in suitable volatile solvents in which the binding material employed is also dissolved or incorporated, the binding material preferably comprising colloidal or protective material giving the desired strength or body to the leaf and also protecting the tinting and coloring material incorporated therein. Resinous gums, such as copal, sandarac, mastic, and so forth, may be used for the binding and protective material, together with more or less soluble cellulose, such as acetyl or nitrated cellulose or the like, all being dissolved in suitable volatile organic solvents therefor, such as wood, grain or amyl alcohol, or their esters, such as amyl acetate, or acetone, or other ketones, ethers, and so forth. It is also desirable for many purposes to employ in the compositions suitable softening material properly coöperating with the binding or protective material so as to insure the desired pliability and toughness of the leaf and also in some cases to promote its adhesive properties when stamped or otherwise applied to the sized or even unsized surfaces. Camphor or other unctuous, that is, pliable waxy material acting in a generally similar way is desirable for this purpose and seems to minimize adhesion of the leaf to heated embossing book-binding tools, for instance. In producing duplex metallic leaf as above described in which the finished leaf has a tinted or gold appearance on one side and a lustrous silver appearance on the other side due to the stratification of powdered aluminum adjacent thereto, it is desirable to have the solvents of such character and present in such proportion as to facilitate this stratifying action, for which reason also the finely divided metallic coloring matter, such as finely divided aluminum powder, for instance, should not be present in excessive proportions.

A suitable illustrative composition for this purpose may comprise four ounces of soluble cotton and three to four ounces of gum camphor dissolved in one gallon of the volatile solvent which may be formed of substantially equal parts of amyl acetate, of benzine and of denatured or grain alcohol, the solution being preferably effected first

in the amyl acetate. When a homogeneous solution of the protective and softening material has been effected the tinting material may be incorporated therewith as by dissolving about one and one-half ounces of naphthalene yellow in a gallon of this composition and then stirring in so as to thoroughly incorporate therewith about ten ounces of finely divided aluminum powder to make a homogeneous composition which preferably soon after its preparation should be sprayed or otherwise applied to the backing material to form the leaf.

Another illustrative composition may be formed by dissolving three to four ounces of camphor and one to three ounces of sandarac and two to three ounces of acetyl or nitrated cellulose in a gallon of a suitable volatile solvent therefor, such as a mixture of one-third to one-half of amyl acetate with diacetone alcohol, benzol or benzin. And in incorporating with a gallon of such solution about two ounces of naphthalene yellow or auramin and one-half ounce of gum gamboge and uniformly dissolving such tinting material therein and then incorporating about ten ounces of aluminum powder with the composition when deeper gold leaf is desired.

Other illustrative liquid binding compositions or carrier liquids are indicated in my former Patents 976,994 of November 29, 1910 and 984,805 of February 21, 1911, which also describe in some detail the general method of making leaf of this description as by spraying or otherwise applying the compositions to sized backing paper or other fabric and separating the dried decorative leaf from the backing by suitable solution of the sizing material. In making metallic decorative leaf such as the duplex metallic leaf or other imitation gold leaf, it is desirable to quickly and uniformly apply the metallic compositions and form a layer thereof which can be allowed to dry under uniform conditions so as to promote and effect the desired stratification in manufacturing duplex leaf of this character. For these reasons it is desirable to spray the composition uniformly upon the sized paper backing or other support and then effect the drying of the applied layer under such conditions as to allow the stratification of the dissolved tinting and protective material adjacent the sized surface of the backing, for instance, which usually takes place with such illustrative compositions within one or several minutes or so, even a minute being sufficient for some of these compositions to separate or stratify to the desired extent through the unusual surface tension or other physical or quasi-chemical action which seems to take place. A layer of yellowish composition of this character comprising incorporated powdered aluminum which looks distinctly

yellow when first sprayed upon the sized paper backing will turn to a distinctly silvery color within a minute or so if allowed to dry slowly. While if the drying of the volatile solvents is hastened by additional heat or by forced air currents the original yellowish color of the freshly applied layer is maintained so as to be present in the fully dried leaf which is thus substantially uniformly yellowish or golden colored on both sides when removed from the backing. When, however, the stratification is effected as seems desirable in making this duplex metallic leaf the dissolved tinting and protective material seems to stratify adjacent the size backing which thus gives a smooth or burnished surface to this yellowish face of the leaf which also has a metallic luster, thus closely imitating gold leaf and making the leaf when used with this gold colored face outward suitable imitation gold leaf for bookbinding and many other purposes and also having the important advantage that it is practically free from the discoloration or staining produced by many kinds of leather on many kinds of artificial gold leaf comprising bronze powder or the like. The stratification referred to also gives a much thicker layer or coating of protective material above the metallic coloring matter of the leaf under these conditions so that for many purposes it is unnecessary to apply to this face of the leaf any additional protective layer or coating, although if desired an additional coating of impervious or colloidal material may be applied to this gold colored face of the duplex leaf where it is to be used under especially severe conditions. If desired also the reverse or silver colored face of the duplex leaf may be similarly protected by an additional impervious or protective coating preferably comprising colloidal material which may of course be sprayed upon the dried leaf before it is removed from the backing material. For many purposes, however, it is unnecessary to apply any such additional protective layers to the duplex leaf which can thus be formed on the backing in a single operation, the unitary body of the leaf comprising sufficient protective material to prevent undesirable action on the metallic coloring matter which for use on leather goods should preferably be powdered aluminum metallic coloring matter or such similar powdered coloring matter as is permanent against leather compositions. The protective material also serves to give the leaf sufficient strength and also serves to make the leaf adherent to cloth, leather or other material to which it is applied and good adhesion can be readily secured when such leaf is stamped with slightly heated dies or embossing tools especially when the leaf body comprises camphor or other softening ma-

terial which seems to promote clean and desirable stamping action.

- It is of course understood that one or more faces of the duplex or other metallic leaf may be given a different tint or color by employing in connection therewith different coloring matter, such for example, as crystal violet, safranin, eosin, fuchsin, Bismarck brown, and so forth which can be used in about the same proportions as the yellowish tint or coloring matter previously suggested for use where a gold colored face is to be formed on the duplex leaf. If desired also these or other colors may be separately applied or sprayed upon the body of the leaf so as to give the desired tint with or without metallic luster, preferably in connection with the aluminum or other permanent powdered coloring matter used in the leaf body. In this way the desirable permanence or non-staining, non-oxidizing properties can be secured in the decorative leaf so as to make it practically free from discoloration or staining such as is caused when staining or oxidizing metal powder is used in the leaf body. Any leaf of this general description may be provided with an incorporated sizing coating so as to make it adherent under ordinary embossing conditions by spraying the leaf body with a suitable sizing, such for example as a solution of about a pound of gum shellac or other suitable gum in a gallon of wood alcohol or other suitable solvent. In this way the sizing is localized on the surface of the leaf, although it is of course apparent that suitable sizing composition may be otherwise incorporated with the leaf so as to obviate the special sizing operation sometimes used in applying such leaf.

This invention has been described in connection with a number of illustrative ingredients, compositions, formulas, proportions and methods of operation, to the details of which disclosure the invention is not of course to be limited, since what is claimed as new and what is desired to be secured by Letters Patent is set forth in the appended claims.

50 I claim—

1. The duplex metallic decorative leaf having a body comprising colloidal protective and binding material including cellulose ester and incorporated powdered aluminum metallic coloring matter, and incorporated dissolved organic yellow tinting material stratified adjacent one side of said duplex leaf to form a gold colored face thereon, the metallic coloring matter being stratified adjacent and more clearly visible from the other side of said leaf to form a silver colored face thereon.
2. The duplex metallic decorative leaf having a body comprising colloidal protective and binding material and incorporated

aluminum metallic coloring matter, and incorporated yellow tinting material stratified adjacent one side of said duplex leaf to form a gold colored face thereon, the metallic coloring matter being stratified adjacent and more clearly visible from the other side of said leaf to form a silver colored face thereon. 70

3. The thin pliable duplex metallic decorative leaf having a body comprising colloidal protective and binding material and incorporated powdered white metallic aluminum coloring matter, and incorporated dissolved organic yellow tinting material stratified adjacent one side of said duplex leaf to form a gold colored face thereon, the metallic coloring matter being more readily visible from the other side of said leaf to form a silver colored face thereon. 75 80

4. The thin pliable duplex metallic decorative leaf having a body comprising protective and binding material and incorporated powdered white metallic coloring matter, and incorporated tinting material stratified adjacent one side of said duplex leaf to 85 form a gold colored face thereon, the metallic coloring matter being more readily visible from the other side of said leaf to form a silver colored face thereon. 90

5. The artificial gold leaf practically free from discoloration from ordinary leather on which it may be used, having a substantially burnished face and a body comprising protective or binding material, incorporated powdered metallic aluminum coloring matter and incorporated dissolved organic yellow tinting material stratified adjacent the face of said leaf to produce a gold colored lustrous metallic appearance in connection with the metallic coloring matter. 95 100 105

6. The artificial gold leaf practically free from discoloration from ordinary leather on which it may be used, having a substantially burnished face and a body comprising protective or binding material, incorporated metallic aluminum coloring matter and incorporated organic yellow tinting material stratified adjacent the face of said leaf to produce a gold colored lustrous metallic appearance in connection with the metallic coloring matter. 110 115

7. The artificial gold leaf having a body comprising protective or binding material, incorporated metallic aluminum coloring matter and incorporated tinting material stratified adjacent the face of said leaf to produce a gold colored appearance in connection with the coloring matter. 120

8. The artificial gold leaf practically free from discoloration from ordinary leather on which it may be used, having a body comprising protective or binding material, incorporated powdered aluminum metallic coloring matter and incorporated organic yellow tinting material stratified adjacent 125 130

the face of said leaf to produce a gold colored lustrous metallic appearance in connection with the metallic coloring matter.

9. The artificial gold leaf practically free from discoloration from ordinary leather on which it may be used, having a body comprising protective or binding material, incorporated powdered white metallic color-

ing matter and incorporated tinting material to produce a gold colored lustrous metallic appearance in connection with the metallic coloring matter. 10

JULIUS A. C. FICHTMUELLER.

Witnesses:

JESSIE B. KAY,  
ALBERT E. THAYER.